

Nov. 20, 1956

W. K. VAN ORMER ET AL

2,770,928

ABRASIVE ARTICLE

Filed June 15, 1951

3 Sheets-Sheet 1



FIG. 1



FIG. 2



FIG. 3

INVENTOR.

WILLIAM K. VAN ORMER

JOSEPH B. AUST

BY *W. K. Dolay*  
ATTORNEY

Nov. 20, 1956

W. K. VAN ORMER ET AL

2,770,928

ABRASIVE ARTICLE

Filed June 15, 1951

3 Sheets-Sheet 2



FIG. 4



FIG. 5



FIG. 6



FIG. 7



FIG. 8

INVENTOR.

WILLIAM K. VAN ORMER

JOSEPH B. AUST

BY   
ATTORNEY

Nov. 20, 1956

W. K. VAN ORMER ET AL

2,770,928

ABRASIVE ARTICLE

Filed June 15, 1951

3 Sheets-Sheet 3



FIG. 9

INVENTOR.  
WILLIAM K. VAN ORMER  
JOSEPH B. AUST  
BY *W. K. Van Ormer*  
ATTORNEY

1

2,770,928

## ABRASIVE ARTICLE

William K. Van Ormer and Joseph B. Aust, Niagara Falls, N. Y., assignors to The Carborundum Company, Niagara Falls, N. Y., a corporation of Delaware

Application June 15, 1951, Serial No. 231,744

9 Claims. (Cl. 51—195)

This invention relates to abrasive articles of manufacture such as abrasive discs, belts, bands, wheels and other forms of abrasive articles.

Abrasive products can be usually classified or identified with one or the other of two broad classifications of abrasive products, namely, those belonging in the field of bonded abrasive bodies of the grinding wheel type consisting of a substantial bulk of abrasive grains and bond and those belonging in the field of coated abrasives of the sandpaper type in which a substantially single layer of abrasive grains is adhesively secured to a flexible backing material. Each of these types of abrasive products has certain advantages not possessed by the other type as well as certain limitations.

In the manufacture of bonded abrasive articles of the grinding wheel type the individual abrasive particles are bonded together by means of an organic or inorganic binder, the desired body being formed by mixing the abrasive grains and bond together to form a molding mixture which is then pressed or otherwise formed into a solid mass of material of the desired shape. The article is then heated or fired to mature the bond and form the desired solidified rigid mass which is then usually dressed to size. The resulting rigid body of abrasive material is either cemented or bolted to a steel backing plate or other support or mounted conventionally on a machine shaft or spindle with appropriate bushings or flanges and operated at relatively high speeds to perform the desired abrading operation.

The strength of the bonded abrasive body is dependent to a great extent upon the strength of the fired or cured bonding material and is controlled within certain limits by the amount by weight and volume of the bonding material in relation to the total weight and volume of the bonded abrasive body. The resultant article is rigid, non-flexible and normally quite brittle and therefore requires careful testing before use. Precautions must be taken in respect to its mounting and use in order to provide the maximum degree of safety during its operation at relatively high speeds. The inherent rigidity, accompanied as it is by a relatively high degree of brittleness or fragility, greatly restricts the scope of application of such articles.

However, products of the grinding wheel type offer the prime advantage of having relatively long operating lives. A further advantage is the relatively high rate of breakdown or expendability which can be tolerated in view of the availability of a substantial amount of abrasive material in the article, and is often desirable to promote a high rate of cut. The rate of wearability or breakdown is dependent largely upon the bond structure of the body which sometimes is rendered porous by the incorporation of filler materials which are volatilized or burned off during the maturing of the bond, particularly in wheels which are designed for fast cutting operations and relatively rapid wheel breakdown is desired. A grinding wheel which cuts fast is referred to as a "soft" wheel and wears away relatively rapidly. However, pro-

2

motion of the porosity and rate of cut of a wheel in the above manner has its limitations since it is accompanied by a lowering of wheel strength and life.

In contrast to abrasive products of the grinding wheel type which are extremely hard, rigid and inflexible in character and have relatively long operating life, abrasive articles of the coated type consist of a substantially single layer of abrasive grits adhesively secured to a flexible backing and, as a result of the relatively small amount of abrasive particles available in the article, the products have a relatively short life with a very high rate of stock removal. Consequently, the cost of various backing materials in such products must be kept to a minimum in order that the overall cost of the product does not become so great as to nullify the advantages gained from the flexibility and versatility of the products derived therefrom. Attempts to extend or prolong the life of coated abrasive products by the use of heavier coatings of abrasive material in conjunction with the use of extra heavy or more durable backings have never proven satisfactory since such products have tended to become dull and glazed regardless of coating thickness and often break down excessively due to the premature separation of the abrasive coating from the backing.

It is an object of the present invention to provide abrasive articles which combine to a large extent the long operating life and durability of abrasive articles of the grinding wheel type with certain elements of versatility and flexibility previously found only in abrasive articles of the coated abrasive or sandpaper type.

It is a further object to provide a type of abrasive article which can be made with any desired degree of rigidity or flexibility.

It is a further object to provide abrasive products having a relatively substantial mass of abrasive material embodied in the article without total loss of flexibility characteristics.

It is a still further object to provide an abrasive product in which a substantial mass of bonded abrasive material is embodied in the article and secured to a supporting structure in such a manner that the abrasive mass is substantially fully expendable without premature disruption or dislocation from its support.

These and other objects and advantages accruing from the present invention will become apparent as the description proceeds.

In order that the invention may be more fully understood, reference is made to the drawings which are offered by way of illustration only, are not intended to restrict the invention in any way to the specific articles shown, and in which,

Figure 1 is a top plan view of an abrasive disc made in accordance with the present invention,

Figure 2 is a vertical, diametrical cross-sectional view through the line 2—2 of Figure 1,

Figure 3 is a vertical, sectional view through an endless abrasive belt made in accordance with the present invention,

Figure 4 is a vertical, diametrical sectional view through a cup-shaped abrasive wheel made in accordance with and embodying various features of the present invention,

Figure 5 is a view similar to that of Figure 2 of a modified form of abrasive disc embodying features of the present invention,

Figure 6, likewise similar to Figure 2 in view, shows a still further modification of the invention,

Figure 7 shows certain structural details of the textile anchoring layer and vertical pile members embodied in the disc structure shown in Figure 2 and the belt structure shown in Figure 3,

Figure 8 shows a top plan view of a modified form of abrasive disc; and

Figure 9 is a graph showing graphically the grinding results obtained with products of the present invention as compared to conventionally prepared coated abrasive articles and bonded articles heretofore used for the same purpose.

We have found that abrasive articles such as abrasive discs, wheels, belts, bands and other shapes can be made in accordance with and embodying various features of the present invention so as to combine the long life and durability characteristics in many respects found in abrasive articles of the grinding wheel type with that flexibility and dependent versatility of application heretofore found only in coated abrasive products. The invention is not intended to be limited to the specific articles illustrated in the various figures of the drawing since it is applicable to the construction of numerous forms of abrasive articles commonly known and used in the art including such articles as:

1. Abrasive bands and belts for operating over either drums or pulleys and back-up plates,
2. Abrasive discs for use with or without auxiliary back-up supports,
3. Cup wheels,
4. Annular type snagging wheels,
5. Ring and recessed wheels of various types and sizes,
6. Flexible polishing wheels; and
7. Blocks and shapes adapted for use on expanding chucks such as those shown in U. S. Patents Nos. 2,207,439 and 2,264,589.

Abrasive articles of the present invention, regardless of their specific form or shape, are provided with a layer of bonded abrasive material of substantial thickness and are further characterized by having a multitude of spaced pile members extending through the mass of bonded abrasive substantially to the grinding surface with the lower ends of the pile members anchored in the base layer of the article in any one of a variety of ways. The article is further characterized in that the bonded abrasive mass provides a substantially continuous or solid grinding surface with no deep, irregular depressions between the spaced pile members contained therein. The reinforcing pile members can be of any material of organic or inorganic nature and can be single or multiple strands, either straight, crimped or looped members, and either filamentary or fibrous in character. For example, the spaced pile members can be composed of various textile fiber cord materials, such as corded cotton fibers, corded wool fibers or other animal or vegetable fibers, or filamentary materials. The pile members can also be composed of any of the numerous synthetic organic materials now available in either fibrous or filamentary form, such as the polyamide fibers or filaments known and sold by E. I. du Pont de Nemours and Company of Wilmington, Delaware, under the generic trade name of "nylon," the vinylidene chloride polymers in fibrous or filamentary form such as those known and sold by Dow Chemical Company of Midland, Michigan, under the trade name of "Saran" fibers or filaments, or by Firestone Plastic Company of Pottstown, Pennsylvania, under the trademark name of "Velon" fibers or filaments, the zein protein fibers known under the trademark name of "Vicara" fibers and sold by the Virginia-Carolina Chemical Corporation, Fiber Division of Taftville, Connecticut, the viscose rayon fibers sold by E. I. du Pont de Nemours and Company under the trade name of "Cordura" fibers, or the polyacrylonitrile fibers sold by the same company under the trade name of "Orlon" fibers, or other organic resinous fibrous or filamentary materials. The pile members can also consist of an inorganic filament or fiber such as a cord or rope composed of glass or rock wool fibers or filaments such as those known and sold by Owens-Corning Fiber-

glas Corporation of Toledo, Ohio as "Fiberglas" products.

These pile members which extend through the mass of granular abrasive material and are an essential feature of articles made in accordance with the present invention are anchored at their lower ends in any one of a variety of ways. For example, the pile members can be secured in the base of the bonded abrasive layer by being set or anchored in a solidified layer of adhesive or binder which is preferably of the permanently flexible or resilient type such as a rubber base adhesive or a coagulated latex adhesive composition. Also various resinous binders of a naturally and permanently flexible type, or a resinous bond which retains its strength under 10 and after mechanical flexing, can be used. The anchoring layer of the article instead of consisting of a layer of adhesive or binder may be, and preferably is, constructed of one or more courses of interwoven warp or braid strands of textile fibrous material which is in 15 turn reinforced and held together by being impregnated with a suitable adhesive, usually of the resilient type, such as a latex or rubber base adhesive composition. Where reference is made to the use of a latex or rubber base adhesive in the anchoring layer it is intended to 20 include not only natural rubber latex or natural rubber base adhesives, but also those various synthetic latices or rubber compositions available such as the butadiene type synthetic rubbers, polychloroprene, and the like. When a layer of textile material is used in the anchoring 25 layer the vertical pile members are anchored therein, such as by being looped through one or more of the courses of warp strands with the free ends of the vertical pile members extending or protruding above the flat surface of the anchoring layer into the bonded abrasive mass which is superimposed thereon. Another manner of providing a plurality of spaced, vertical pile members anchored in a warp or braid strand heading or base is by interweaving a continuous cord or strand through 30 one or more courses of the base layer with loose loops of the cord or strand pulled up and projecting in a loop above the upper face of the base layer at selected intervals. This anchoring layer is usually, although not necessarily, backed up or supported by a further backing layer of 35 flexible nature such as a rubber or latex impregnated sisal fiber backing, a thin sheet of spring steel, vulcanized fiber 40 backing, or the like.

A further and specific modification of the present invention consists in the provision of an article of the above-described type in which a combination of vegetable or animal pile members with pile members of a more heat resistant character, such as pile members of synthetic resinous material such as "nylon" or "Saran" are incorporated within the bonded abrasive layer. Also, 50 combinations of any organic fiber can be used in conjunction with inorganic glass or mineral fibers. The ratio of animal or vegetable fibers or other organic fiber pile members of low heat resistance to "Velon," "nylon," glass or other more heat-resistant pile members can range all the way from 5% to 95% of one to 95% to 55 5% of the other, or any intermediate combination of two or more fibrous or filamentary materials. During the cure of an article embodying a combination of two or more materials as pile members the less heat resistant 60 pile members disintegrate to provide relatively weak areas in the bonded abrasive mass whereby those areas of the overall structure tend to break down more rapidly than adjoining areas. The remaining fibers of more heat resistant character break down later during the 65 grinding operation without interfering with the cutting ability of the article although at the same time they would remain in the body of the abrasive mass as a reinforcing and strengthening element. By the use of such composite mixtures of vertical pile members it is possible to provide a wide range of different desirable cut- 70 75

ting characteristics depending upon the type and condition of use to which the article is to be put.

In practicing the invention, any of the abrasive materials in common use may be employed, such as granular silicon carbide, diamonds, boron carbide, fused aluminum oxide, flint, corundum, emery, rouge and similar substances. Another specific, and relatively new, product which can be used as the abrasive material in articles of the present invention is a foam, or cellular, glass in granulated form. Regardless of the kind of abrasive used, the size of the abrasive particles may vary from the finest polishing or buffing powders to the coarser grit sizes used in grinding.

The abrasive particles can be bonded with any suitable bond which can be matured at temperatures which will not destroy the vertical pile members which are to remain in the finished article as a permanent part thereof and which function to preserve the integrity of the article over its intended life or until the abrasive layer has been usefully expended. Very satisfactory results have been obtained usefully expended. Very satisfactory results have been obtained with the use of thermosetting phenolic condensation product resins, including those specifically set forth later herein in connection with the various examples. However, other organic binding materials, all of which can be modified by the inclusion of suitable catalysts or vulcanizers, inert and reactive fillers, and other modifying agents as desired, can be used.

Among the organic resins which can be used are melamine-formaldehyde resins and analogs thereof, urea-formaldehyde resins and analogs thereof, thiourea-formaldehyde resins and analogs thereof, furane resins, aniline-formaldehyde resins, thermosetting alkyd resins, thermosetting polyesters such as diallyl phthalates, diallyl carbonates, styrene and maleic anhydride-glycol adducts, and the like, and thermosetting bisphenol-epichlorohydrin resins and analogs thereof. The thermosetting bisphenol-epichlorohydrin resins are especially useful where it is desired to form a bonded abrasive mass in which the bond will set to a hardened condition at room temperature without the application of heat.

Other substances which can be used as the bond for the abrasive particles include shellac, natural rubber and the various synthetic rubbers, such as butadiene-styrene copolymers, butadieneacrylic nitrile copolymers, polychloroprene and the like. An inorganic bond which can be used is an air-setting hydraulic cement such as magnesium oxychloride.

The various materials set forth above as bonding substances for the abrasive particles can be used in the form of suitable liquids, solutions, emulsions, or dispersions, depending upon the form in which the bonding material is most economically available.

Referring further to various figures of the drawing, Figures 1 and 2 depict an abrasive disc consisting of a layer 8 of bonded granular abrasive material of substantial thickness, as for example in the order of magnitude of  $\frac{1}{8}$ " in thickness, adhesively secured to a textile anchoring layer 9 which in turn is adhesively bonded to a backing 10 of latex-impregnated sisal fiber. The bonded abrasive layer 8, as shown in Figure 1, has a plain continuous flat upper grinding surface 12. However, the disc can be modified, when desired, by pressing the abrasive layer with a top plunger having a gridded surface whereby the upper grinding surface 12 of the abrasive layer 8 is provided with a plurality of shallow annular grooves 13 and a plurality of radial grooves 24, such a modified form of disc being illustrated in Figure 8.

Referring to Figure 7 for further details of the textile layer 9 it can be seen that this element of the article which can be referred to as the anchoring layer or "heading" comprises a single course 11 of interwoven warp or braid strands of textile fibrous material such as cotton strands which are spirally wound and impregnated with a latex adhesive composition to form an annular resilient sup-

porting surface for the bonded abrasive layer and also as a means for mechanically anchoring the vertical pile members 14 which, as shown in Figure 7, are looped through the layer of interwoven textile warp strands 5 with the free ends 15 extending vertically above the anchoring layer of warp strands a distance substantially equal in thickness to the thickness of the bonded abrasive layer. As clearly pointed out these vertical pile members can consist of any organic or inorganic fibrous or 10 filamentary material, or combinations of one or more organic fibrous or filamentary materials with one another or with inorganic fibrous or filamentary materials. The central or arbor portion of the abrasive disc shown is further reinforced by a centrally positioned disc 16 which 15 is also of latex-impregnated compressed sisal fibers. The abrasive disc is provided with a mounting arbor hole 17 of suitable diameter for mounting upon the driving spindle or shaft of the machine upon which the abrasive disc is to be used. The vertical pile members 14 not only 20 strengthen and reinforce the bonded abrasive layer of the article throughout its thickness but, anchored as they are in the textile base layer 9 of the article, they also serve to prevent disruption or dislocation of the bonded abrasive layer from its supporting base or anchoring layer during 25 the use of the article. The inherently flexible and resilient character of the backing 10 and the anchoring layer 9 provide in the finished product a degree of flexibility and resilience utterly lacking in a conventional abrasive article of the grinding wheel type while at the same time the 30 substantial thickness of bonded abrasive material provided in the article provides a useful life far exceeding that to be found in similar abrasive articles of the conventional coated abrasive type.

Figure 3 shows an endless abrasive belt consisting of 35 a flexible backing 18 to which is bonded a textile anchoring layer 19, which latter layer comprises a single course of interwoven textile warp or braid strands similar to the warp strand course embodied in the anchoring layer of the disc of Figures 1 and 2. This warp strand anchoring 40 layer is impregnated with a latex base adhesive which secures the anchoring layer to the backing 18 and also provides additional strength and resilience to the anchoring layer itself. A multitude of spaced vertical pile members 20 of twisted "nylon" cords are looped through the 45 warp strands in a manner such as that shown in Figure 7 and extend above the top surface of the anchoring layer. The space between the vertical pile members 20 is filled with a thick layer 21 of bonded abrasive material such as a mixture of abrasive granules and phenolic resin bond. 50 Before use the belt is flexed over a small diameter steel rod or bar to fracture the coating of abrasive material 21 transversely of the belt in a plurality of places 22 so that the abrasive belt can be rotated upon a drum or set of pulleys although at the same time the belt presents 55 a substantially continuous grinding surface 23 to the work to be abraded. Each fragment of the belt however contains a number of vertical pile members which act as a means of securing the separate fragments of the abrasive 60 coating against shearing away from the anchoring layer.

Figure 4 shows a cup wheel which is composed of a bonded abrasive body 25 reinforced by a multitude of spaced vertical pile members 26 which are anchored in a textile anchoring layer 27 which is in turn cemented 65 to the mounting hub 28. The mounting hub, which can be of aluminum or other metal, a molded resin body, or other suitable structural material, is provided with a screw threaded arbor hole 29 suitable for mounting the abrading device upon a spindle or shaft. The textile anchoring layer 27 is composed of a single course of interwoven warp or braid strands similar to the structure shown for the anchoring layer of the abrasive belt pictured in Figure 3. However, it may consist of one or 70 more courses of a coarsely woven textile fabric such as glass fiber fabric, burlap, canvas, or the like, through 75

which the pile members 26 are needled or looped to anchor them in the textile layer.

Figure 5 shows a modified form of abrasive disc in which the bonded abrasive body 31 extends over the entire upper face of the disc, and in which the spaced vertical pile members 32 are anchored in an anchoring layer 33 of a rubber base adhesive by which the bonded abrasive body is adhesively secured to the backing or support 34.

Figure 6 shows a still further modification of the invention in the form of an abrasive disc in which the abrasive body 36 is reinforced by vertical pile members 37 which are anchored in a base layer 38 of latex-impregnated interwoven textile warp strands similar to those described for Figures 1 and 2. This particular modification of the invention is for use in conjunction with a separately provided back-up pad or plate and therefore is not provided with a backing support as a permanent part of the article.

Abrasive articles of the above-illustrated type, as for example the abrasive disc shown in Figures 1 and 2 have been made in the following manner.

#### Example I

A disc shaped base was provided consisting of an anchoring layer or "heading" of a single interwoven, spirally laid course of cotton warp strands which is impregnated with latex and thereby cemented to a  $\frac{1}{8}$ " thick latex-impregnated sisal fiber backing. The anchoring layer had a plurality of spaced vertical pile members consisting of 50% twisted cotton fiber cording and 50% twisted "Saran" fiber cording looped through the interwoven strands of the warp or braid strand course and spaced approximately  $\frac{1}{4}$ " from one another circumferentially and about  $\frac{1}{16}$ " from one another radially of the disc, although any other desired degree of spacing of the pile members, either more open or closer together, may be employed, if desired. The vertical pile members extended approximately  $\frac{1}{8}$ " above the upper face of the warp strands. The upper surface of the anchoring layer as thus provided was dip-sized with a low-viscosity, phenol formaldehyde liquid resin containing 1/2% of a wetting agent. One suitable phenol formaldehyde liquid resin found suitable for sizing was that known and sold by the Bakelite Corporation of Bloomfield, New Jersey, under the trademark designation of Bakelite No. BR10190 resin. A suitable wetting agent is that known and sold under the trademark name of "Span 20" by Atlas Powder Company of Wilmington, Delaware. "Span 20" is otherwise identified as sorbitan monolaurate. The sized disc was then placed in a die mold and an abrasive mixture of the following composition applied to the top surface of the disc in sufficient quantity to fill the space between the spaced vertical pile members and levelled off flush with the tops of the vertical pile members:

|                                                                                 | Grams |
|---------------------------------------------------------------------------------|-------|
| Low-viscosity, phenol formaldehyde liquid resin<br>(such as "Bakelite BR10190") | 300   |
| Calcium carbonate                                                               | 200   |
| Ethylene glycol                                                                 | 30    |
| Sorbitan monolaurate (such as "Span 20")                                        | 1.5   |
| Sorbitol                                                                        | 5     |
| 24 grit size, fused alumina abrasive grain                                      | 1000  |

A surface coating of loose abrasive grain of the same grit size and character was applied to the top surface of the abrasive coated disc after which the disc was placed under light pressure sufficient to seat the entire abrasive mass firmly. The disc was then placed in an oven and subjected to the following heat treatment to mature the resin bond: 24 hours at 135° F., 2 hours at 150° F., 18 hours at 175° F., 2 hours at 185° F., 18 hours at 200° F., 2 hours at 225° F., 12 hours at 250° F., 3½ hours at 275° F., and 4 minutes at 375° F. The oven

was then allowed to cool to room temperature and the abrasive disc removed ready for use.

#### Example II

Abrasive discs of the type shown in Figures 1 and 2 have been made as follows: A disc shaped base of the type described in Example I was provided, the sole difference being that the spaced vertical pile members consisted entirely of twisted cotton cording, although the pile members were spaced the same as those in Example I. The upper or piled surface of the heading was first dip-sized with a low viscosity, phenol formaldehyde liquid resin such as that used for the same purpose in Example I. The sized disc was then placed in a mold and an abrasive mixture of the following composition applied to the top surface of the disc and rolled into the spaces or recesses between the pile members in increments until the pile members were covered with sufficient abrasive-bond mixture to bring the top surface of the mass, when levelled off, flush with the tops of the vertical pile members.

|                                                                                                                       | Grams |
|-----------------------------------------------------------------------------------------------------------------------|-------|
| Low viscosity, phenol formaldehyde liquid resin<br>(such as that known and sold under the name<br>"Bakelite BR10190") | 341   |
| Calcium carbonate                                                                                                     | 426.4 |
| Ethylene glycol                                                                                                       | 76.7  |
| Sorbitan monolaurate (such as that known and sold<br>as "Span 20")                                                    | 3.8   |
| 24 grit size, fused aluminum oxide abrasive grain                                                                     | 935   |

The disc was pressed at 4000 pounds per square inch and placed in an oven and subjected to the following heat treatment to mature the resin bond: 6 hours at 130° F., 15 hours at 150° F., 6 hours at 170° F., 2½ hours at 185° F., 18 hours at 200° F., 12 hours at 225° F., 6 hours at 250° F., and 3½ hours at 275° F. Temperature taken to 350° F. after which the oven was allowed to cool to room temperature immediately and the discs removed ready for use.

The resulting abrasive disc made as above-described was used to grind welds from metal surfaces with the following results. The disc was operated for a total grinding time of 69 minutes during which time a typical abrasive disc removed a total of 4345 grams of metal with a disc weight loss of 335.9 grams. This can be compared to the results obtained with a conventional 24 grit size resin bonded sander disc made by prior art methods in which the disc was operated for a total time of 21 minutes before failure with a total metal stock removal of 715 grams. A cup wheel removed 3392 grams of metal in 54 minutes at a rate of 62.7 grams per minute and a wheel loss of 906.5 grams at 5400 R. P. M. The grinding results obtained with an abrasive disc made according to Example II as compared to the grinding results obtained with a conventional resin bonded abrasive coated disc of the same abrasive grit size and a resin bonded cup wheel are shown in Figure 9. As the graph shows, the life of the sander disc (see curve A of graph) is inordinately short as compared to the period of usefulness shown by an abrasive disc made according to the present invention (see curve B of graph) and even compares favorably with the long life of the rigid bonded cup wheel (see curve C of graph). The actual cutting rate of the abrasive disc as herein made is also noted as being remarkably high, averaging 63 grams of metal removed per minute over the entire 69 minutes grinding period of the test. The remarkably longer life and durability of discs made in accordance with the present invention as compared to conventional abrasive coated discs heretofore used for the same purpose is outstanding.

Inasmuch as the term "braided" is sometimes narrowly construed to refer to a type of cording made up from a plurality of intertwined strands, it is to be pointed out that where the term "braided" is used herein it is intended to refer not only to cording made up from a plurality of

intertwined strands, but also to cording made up from a single strand interlocked with itself in such a manner as to form a cording of braided appearance, such as that shown in Figure 7.

Having described the invention it is desired to claim:

We claim:

1. An abrasive disc comprising a backing and a substantially continuous layer of bonded abrasive material secured thereto, said backing comprising a base layer, a textile fiber layer comprising at least one spirally wound braided strand forming an anchoring layer upon said base layer and adhesively bonded thereto, and a multitude of spaced vertical reinforcing pile members passing through said braided strand and extending into the aforesaid layer of bonded abrasive material.

2. An abrasive disc comprising a backing and a substantially continuous layer of bonded abrasive material secured thereto, said backing comprising a base layer of latex-impregnated sisal fiber, a textile fiber layer comprising at least one spirally wound braided strand forming an anchoring layer upon said base layer and adhesively bonded thereto by means of a latex base adhesive, and a multitude of spaced vertical reinforcing pile members passing through said braided strand and extending into the aforesaid layer of bonded abrasive material.

3. An abrasive article comprising (a) a backing, (b) an anchoring layer comprising at least one course of textile fiber braided strand adhesively impregnated and bonded to said backing by means of a flexible rubber base adhesive and containing a plurality of vertically extending spaced textile fiber reinforcing pile members secured therein with the free ends projecting above the top surface of said anchoring layer, and (c) a layer of resin-bonded abrasive material imposed upon said anchoring layer and filling the space between said spaced pile members so as to form a substantially continuous grinding face.

4. An abrasive article comprising a composite backing comprising a flexible sheet backing material and an anchoring layer of textile braided strand impregnated with a resilient latex base adhesive, said anchoring layer having a plurality of spaced reinforcing pile members anchored therein with the free ends extending vertically therefrom, and a substantially continuous layer of phenolic resin-bonded granular abrasive material bonded to said anchoring layer and of a thickness at least coextensive with the height of said pile members.

5. An abrasive article comprising a composite backing comprising a flexible sheet backing material and an anchoring layer of interwoven textile material impregnated with a resilient latex base adhesive, said anchoring layer having a plurality of spaced reinforcing pile members anchored therein with the free ends extending vertically

therefrom, and a substantially continuous layer of resin-bonded granular abrasive material bonded to said anchoring layer and of a thickness at least coextensive with the height of said pile members.

5 6. An abrasive article according to claim 5 in which the vertical reinforcing pile members are nylon cords and the textile material is a cotton fabric.

7. An abrasive article according to claim 4 in which 10 5% to 95% of said pile members are of heat resistant organic thermoplastic material and 95% to 5% of said pile members are of natural organic fibrous material.

8. An abrasive disc comprising a backing, a substantially continuous layer of bonded abrasive material secured thereto, and a multitude of spaced vertical reinforcing pile members extending into the layer of bonded abrasive material, said backing comprising a single spirally wound braided strand, said pile members passing through said braided strand.

15 9. An abrasive disc comprising a backing, a substantially continuous layer of bonded abrasive material secured thereto, and a multitude of vertical reinforcing pile members extending into the layer of bonded abrasive material, said backing comprising at least one spirally wound braided strand, said pile members being spaced approximately  $\frac{1}{4}$  inch from one another circumferentially and about  $\frac{1}{16}$  inch from one another radially of the disc and passing through said strand.

References Cited in the file of this patent

| UNITED STATES PATENTS |                           |                |
|-----------------------|---------------------------|----------------|
| 30                    | 1,077,143 Krug            | Oct. 28, 1913  |
|                       | 1,209,831 Gardner         | Dec. 26, 1916  |
|                       | 1,529,410 Doermann        | Mar. 10, 1925  |
| 35                    | 1,775,631 Carlton         | Sept. 16, 1930 |
|                       | 1,822,856 Dirkes          | Sept. 8, 1931  |
|                       | 1,850,413 Porte           | Mar. 22, 1932  |
|                       | 1,899,959 Happ            | Mar. 7, 1933   |
|                       | 1,961,911 Pusch           | June 5, 1934   |
| 40                    | 2,001,911 Wooddell et al. | May 25, 1935   |
|                       | 2,013,925 Okie            | Sept. 10, 1935 |
|                       | 2,071,563 Newcomb et al.  | Feb. 23, 1937  |
|                       | 2,085,211 Budds et al.    | June 29, 1937  |
| 45                    | 2,115,897 Wooddell et al. | May 3, 1938    |
|                       | 2,137,305 Perazzoli       | Nov. 22, 1938  |
|                       | 2,186,001 Bartling        | Jan. 9, 1940   |
|                       | 2,189,754 Cherrington     | Feb. 13, 1940  |
| 50                    | 2,232,389 Jurkat          | Feb. 18, 1941  |
|                       | 2,328,998 Radford         | Sept. 7, 1943  |
|                       | 2,347,244 Colt et al.     | Apr. 25, 1944  |
|                       | 2,520,763 Goepfert et al. | Aug. 29, 1950  |
|                       | 2,590,697 Grove           | Mar. 25, 1952  |

UNITED STATES PATENT OFFICE  
CERTIFICATE OF CORRECTION

Patent No. 2,770,928

November 20, 1956

William K. Van Ormer et al.

It is hereby certified that error appears in the printed specification of the above numbered patent requiring correction and that the said Letters Patent should read as corrected below.

Column 5, lines 20 and 21, strike out "Very satisfactory results have been obtained usefully expended."; column 6, line 49, for "branules" read -- granules --; column 10, line 27, before "strand" insert -- braided --.

Signed and sealed this 15th day of July 1958.

(SEAL)

Attest:

KARL H. AXLINE

Attesting Officer

ROBERT C. WATSON  
Commissioner of Patents